# EUROPEAN PATENT SPECIFICATION

(11) **EP 1 252 353 B1**
(45) Date of publication and mention of the grant of the patent: **16.07.2003**
(21) Application number: 00989092.2
(22) Date of filing: 15.12.2000
(51) Int. Cl.: C22C 37/04, C22C 33/10, C21C 1/08

(54) **NEW ALLOY AND METHOD FOR PRODUCING SAME**
NEUE LEGIERUNG UND HERSTELLUNGSVERFAHREN DAFÜR
NOUVEL ALLIAGE ET PROCEDE DE PRODUCTION CORRESPONDANT

(30) Priority: 17.12.1999 SE 9904668
(43) Date of publication of application: 30.10.2002
(73) Proprietor: SinterCast AB, 100 55 Stockholm (SE)
(72) Inventor: TROSCHEL, Wolfgang, 35578 Wetzlar (DE); TÖLLER, Ralf, 37480 Leon, Guanajuato (DE)
(74) Representative: Bergstrand, Mikael Gudmundsson
(86) International application number: SE0002550
(87) International publication number: WO01044530

(56) References cited:
- SE-C2- 512 201
- US-A- 4 874 576

## Description

The present invention relates to a novel magnesium-treated cast iron containing manganese sulfide (MnS) or molybdenium sulfide (MoS₂) inclusions. The invention also relates to a procedure for preparing the novel cast iron, cast iron products comprising the novel cast iron, as well as using the novel iron for manufacturing cylinder blocks, cylinder heads, bedplates, transmission housings, axle housings or brake drums and discs.

### Technical background

Magnesium treated cast irons, such as compacted graphite iron (CGI) and ductile cast iron (SG) are widely used for a variety of applications. Unfortunately, however, in comparison to conventional grey cast iron these alloys are relatively difficult to machine. This factor has prevented their application to many high volume products which require large amounts of machining. One example is automotive cylinders blocks.

Although the higher strength, stiffness and ductility of CGI and SG relative to conventional grey cast irons accounts for much the difference in machinability between these materials, other factors may also be active. One such factor is the presence of 1-5 µm diameter manganese sulfide (MnS) inclusions in grey cast iron. These inclusions are known to adhere to the cutting edge of the machining tools, thus forming a protective layer and reducing tool wear. The effect is particularly significant at high cutting speeds (400-1 000 m/min) when using cubic boron nitride (CBN) or ceramic cutting materials. It is also known that high sulfur and manganese additions improve the machinability of steels. Such steel alloys are referred to in the trade as "free-machining steels". Again, the mechanism for improved machinability relates to the formation of a protective MnS layer on the cutting insert and/or a lubricating effect of the sulfide inclusions between the cutting insert and the workpiece and/or chip.

Unfortunately, manganese sulfide inclusions are not stable in magnesium-treated cast irons due to the lower free-energy of magnesium sulfide at ironmaking temperatures (Figure 1). Therefore, a previous patent (SE 9800750-3), incorporated by reference, disclosed a method to convert the existing MgO.SiO₂ inclusions in magnesium-treated cast irons to soft calcium-bearing inclusions. However, there are no available methods for producing a magnesium-treated cast iron alloy containing soft and pliable inclusions.

### Summary of the invention

Now, it has surprisingly turned out that it is possible to generate a desirable form (soft, pliable) of sulfide inclusions in magnesium-treated cast irons. Thermodynamically, MnS and MoS₂ are not stable in the presence of magnesium. However, by adding magnesium to a cast iron melt containing manganese sulfide/molybdenium sulfide as late as possible, and preferably when the molten cast iron has been dispensed into the mould, such sulfide inclusions may be preserved in magnesium-treated cast irons. Alternatively, said cast iron can also be formed by adding said sulfides directly to the iron after the magnesium reaction has taken place and an in situ equilibrium has been established between magnesium, oxygen and sulfur. Another option is to begin with a sulfur content in excess of the stoichiometric amount required to combine with the added magnesium, thus ensureing an amount of left-over sulfur to promote the formation of the desired sulfide inclusions.

### Detailed description of the invention.

As disclosed herein, the term "inclusion-forming compound" generally relates to all non-metallic non-organic compounds with hexagonal or face-centred cubic crystal structures and melting points of at least 1100 °C. Preferably manganese sulfide or molybdenium sulfide is used in relation to the present invention.

Accordingly, the present invention relates to a magnesium-treated cast iron containing inclusions which either lubricate the cutting insert or contribute to the formation of a protective layer on the cutting edge of the insert. The inclusions consist of manganese sulfide (MnS) or molybdenium sulfide (MoS₂). Typically, the sulfides are added to a molten base iron as 1 - 100 µm particles. In the presence of heat (1400 - 1500 °C), these particles will become individual spheroids with a uniformly distributed by the convection currents present in the molten iron. This base iron is then treated with magnesium at the last possible moment, preferably when the molten cast iron has been poured into a mould.

The present invention will be disclosed with reference to the enclosed figure 1 which shows temperature dependencies of free precipitation energies ΔGₛ^{o} for some oxides, sulfides, oxysulfides, nitrides and carbides in molten iron.

The theory behind the invention is the following: Prior to the addition of magnesium, an equilibrium will have been established between manganese and sulfur in the base iron as a function of the holding temperature. Once the addition of magnesium is made, the stronger sulfide capacity of the magnesium will reduce the MnS according to the reaction:$\text{MnS +} {\text{Mg}}_{̲} \text{= MgS +} {\text{Mn}}_{̲}$$\text{ΔG° = -73 kJoules/mol at 1 450°C}$

The strongly negative free energy and the exothermic nature of the reaction, combined with the small size, high quantity (approximately 10⁸ MnS inclusions per tonne of liquid iron), suggests that reaction [1] proceeds rapidly to the right. It is therefore important to delay reaction [1] until the last possible moment to prevent reduction of the desired MnS inclusions. Thus, it is proposed that the magnesium addition be made as late as possible, preferably just before the iron is dispensed into the mould or in-the-mould itself.

The process according to the present invention starts with preparing a molten cast iron according to *per se* known methods with a typical base iron chemistry for ductile iron and for compacted graphite iron production:

| | | | |
|---|---|---|---|
| C: | 3.5 - 3.9% | S: | 0.005-0.020% |
| Si | 1.8 - 2.2% | Mn | 0.1-0.5% |

The presence of Mn and S in the base iron will naturally lead to the formation of MnS inclusions according to the thermodynamic equilibrium at the holding temperature. Thereafter, in contrast to typical ductile iron and CGI production techniques which may add the magnesium as much as ten minutes before the start-of-pour, the present invention requires that the molten cast iron is not treated with magnesium until the last possible moment before casting. The magnesium can be added immediately before dispensing the molten iron into the mould, but preferably the magnesium is added to the melt after dispensing the molten iron into the mould. In order to minimise formation of magnesium sulfide after the magnesium addition it is also possible to chill the mould filled with molten magnesium-treated and inclusion-containing cast iron, so that the solidification process is accelerated.

The amount of magnesium added in this step is calibrated in advance. Typically the magnesium content of the final cast iron melt is 0.001 - 0.030% (wt).

Alternatively, a post-addition of MnS particles, or other known solid lubricant particles, namely MoS₂, may be made to the iron after the magnesium reaction has taken place and an in-situ equilibrium has been established between magnesium, oxygen and sulfur. This will allow the MnS or MoS₂ particles to remain in the solidified casting. In this case, 1 - 100 µm manganese sulfide particles of are added. The addition of these particles result in an amount of manganese in the final melt of at least 0.1 % (wt), and typically about 0.6.%. An amount of of about 4 kg manganese sulfide per tonne molten cast iron is typically added, corresponding to 10⁸-10¹² inclusions per tonne molten cast iron, depending on the efficiency of dissolution and assimilation into the melt. A proposed composition for such a master alloy for adding either MnS or MoS₂ particles is as follows:

| | | | |
|---|---|---|---|
| Si | 0-90% | Al | 0-10% |
| Ca | 0-10% | Ba | 0-10% |
| Sr | 0-10% | Zr | 0-10% |
| Re | 0-20% | Mn | 10-90% |
| MnS | 20-70% | MoS₂ | 20-70% |
| Fe | 0 - balance. | | |

Accordingly, this alternative method comprises the steps of a) preparing a molten base iron according to *per se* known methods; b) adding a predetermined amount of magnesium to the molten base iron and allowing establishment of an equilibrium between magnesium, oxygen and sulfur; c) adding a predetermined amount of manganese sulfide and/or molybdenium sulfide; and finally d) casting the melt according to *per se* known methods.

A final option for the stabilisation of MnS in the standard CGI or SG base iron is to increase the sulfur content beyond the typical level of 0.005 - 0.020 % S. In this way, the higher amount of sulfur increases the probability that MnS will form, and indeed survive until the moment of solidification. Thus, the presence of 0.04 % sulfur or more, in the CGI or SG base iron has been shown to result in the presence of MnS inclusions in the final cast products, thus improving their machinability.

## Claims

1. A magnesium-treated cast iron such as compacted graphite cast iron (CGI) or ductile cast iron (SG) containing inclusions of inclusion-forming compounds, which either lubricate the cutting insert or contribute to the formation of a protective layer on the cutting edge, **characterized in that** the inclusions are selected from the group of manganese sulfids (MnS), and molybdenum disulfide (MoS₂).

2. A cast iron alloy according to claim 1, **characterized in that** the desired inclusions are preserved by adding the magnesium alloy at the latest possible moment.

3. A cast iron alloy according to claim 1, **characterized in that** the desired inclusions are preserved by adding the magnesium alloy in-the-mould.

4. A cast iron alloy according to claim 1, **characterized in that** the desired inclusions are formed by adding a master alloy containing the inclusions at the latest possible moment.

5. A cast iron alloy according to claim 1, **characterized in that** the desired inclusions are formed by adding the master alloy in the mould.

6. A cast iron alloy according to claim I, **characterised in that** the desired inclusions are formed by increasing the sulfur content to at least 0.04 %.before casting.

7. A cast iron product comprising an alloy according to claim 1.

8. The use of a cast iron alloy according to claim 1 to produce a cylinder block.

9. The use of a cast iron alloy according to claim 1 to produce a cylinder head.

10. The use of a cast iron alloy according to claim 1 to produce a bedplate.

11. The use of a cast iron alloy according to claim 1 to produce a transmission housing or axle housing.

12. The use of a cast iron alloy according to claim 1 to produce a brake drum or disc.

13. A method for producing a magnesium-treated cast iron containing inclusions, which either lubricate the cutting insert or contribute to the formation of a protective layer on the cutting edge, comprising the steps of:
a) preparing a molten base iron according to *per* se known methods;
b) adding a predetermined amount of magnesium to the molten base iron and allowing establishment of an equilibrium between magnesium, oxygen and sulfur;
c) adding a predetermined amount of manganese sulfide and/or molybdenium sulfide; and finally
d) casting the melt according to *per se* known methods.

14. A method for producing a magnesium-treated cast iron containing inclusions, which either lubricate the cutting insert or contribute to the formation of a protective layer on the cutting edge, comprising the steps of:
a) preparing a molten base iron according to *per se* known methods, said base iron containing at least 0.1 % Mn;
b) increasing the amount of sulfur to at least 0.04 %;
c) adding a predetermined amount of magnesium; and
d) casting the melt according to *per se* known methods.

15. A method according to anyone of claims 13 - 14, further comprising chilling the mould after the casting operation in order to maximise the amount of sulfide inclusions.

## Patentansprüche

1. Magnesiumbehandeltes Gusseisen, wie Kompaktgraphit-Gusseisen (CGI) oder duktiles Gusseisen (SG), mit Einschlüssen von Einschlüsse bildenden Verbindungen, welche entweder den Schneideinsatz schmieren oder zur Bildung einer Schutzschicht an der Schneidkante beitragen, **dadurch gekennzeichnet, dass** die Einschlüsse ausgewählt sind aus der Gruppe der Mangansulfide (MnS) und Molybdändisulfide (MoS₂).

2. Gusseisenlegierung nach Anspruch 1, **dadurch gekennzeichnet, dass** die gewünschten Einschlüsse-erhalten bleiben durch Hinzufügen der Magnesiumlegierung zum spätestmöglichen Zeitpunkt.

3. Gusseisenlegierung nach Anspruch 1, **dadurch gekennzeichnet, dass** die gewünschten Einschlüsse erhalten bleiben durch Hinzufügen der Magnesiumlegierung in der Form.

4. Gusseisenlegierung nach Anspruch 1, **dadurch gekennzeichnet, dass** die gewünschten Einschlüsse gebildet werden durch Hinzufügen einer die Einschlüsse enthaltenden Master-Legierung zum spätestmöglichen Zeitpunkt.

5. Gusseisenlegierung nach Anspruch 1, **dadurch gekennzeichnet, dass** die gewünschten Einschlüsse gebildet werden durch Hinzufügen der Master-Legierung in der Form.

6. Gusseisenlegierung nach Anspruch 1, **dadurch gekennzeichnet, dass** die gewünschten Einschlüsse gebildet werden durch Erhöhen des Schwefelgehaltes auf mindestens 0,04 % vor dem Gießen.

7. Gusseisenprodukt mit einer Legierung nach Anspruch 1.

8. Verwendung einer Gusseisenlegierung nach Anspruch 1 zur Herstellung eines Zylinderblocks.

9. Verwendung einer Gusseisenlegierung nach Anspruch 1 zur Herstellung eines Zylinderkopfes.

10. Verwendung einer Gusseisenlegierung nach Anspruch 1 zur Herstellung einer Bettplatte.

11. Verwendung einer Gusseisenlegierung nach Anspruch 1 zur Herstellung eines Getriebekastens oder eines Achsgehäuses.

12. Verwendung einer Gusseisenlegierung nach Anspruch 1 zur Herstellung einer Bremstrommel oder -scheibe.

13. Verfahren zur Herstellung eines magnesiumbehandelten Gusseisens mit Einschlüssen, welche entweder den Schneideinsatz schmieren oder zur Bildung einer Schutzschicht an der Schneidkante beitragen, umfassend die Schritte:
a) Bereitstellen eines geschmolzenen Basiseisens nach per se bekannten Verfahren;
b) Hinzufügen einer vorgegebenen Menge an Magnesium zu dem geschmolzenen Basiseisen und Einstellenlassen eines Gleichgewichtes zwischen Magnesium, Sauerstoff und Schwefel;
c) Hinzufügen einer vorgegebenen Menge an Mangansulfid und/oder Molybdänsulfid; und schließlich
d) Gießen der Schmelze nach per se bekannten Verfahren.

14. Verfahren zur Herstellung eines magnesiumbehandelten Gusseisens mit Einschlüssen, welche entweder den Schneideinsatz schmieren oder zur Bildung einer Schutzschicht an der Schneidkante beitragen, umfassend die Schritte:
a) Bereitstellen eines geschmolzenen Basiseisens nach per se bekannten Verfahren, wobei das Basiseisen mindestens 0,1 % Mn enthält;
b) Erhöhen des Schwefelgehaltes auf mindestens 0,04 %;
c) Hinzufügen einer vorgegebenen Menge an Magnesium; und
d) Gießen der Schmelze nach per se bekannten Verfahren.

15. Verfahren nach einem der Ansprüche 13 bis 14, ferner umfassend das Kühlen der Form nach dem Gießvorgang zur Maximierung der Menge an Sulfideinschlüssen.

## Revendications

1. Fonte traitée au magnésium, telle que la fonte graphitique compacte (« CGI ») ou la fonte malléable (« SG »), contenant des inclusions de composés formant des inclusions, qui lubrifient l'insert coupant ou contribuent à la formation d'une couche protectrice sur l'arête coupante, **caractérisée en ce que** les inclusions sont choisies parmi le sulfure de manganèse (MnS) et le disulfure de molybdène (MoS₂).

2. Alliage de fonte selon la revendication 1, **caractérisé en ce que** l'on préserve les inclusions désirées en ajoutant l'alliage de magnésium le plus tard possible.

3. Alliage de fonte selon la revendication 1, **caractérisé en ce que** l'on préserve les inclusions désirées en ajoutant l'alliage de magnésium dans le moule.

4. Alliage de fonte selon la revendication 1, **caractérisé en ce que** l'on forme les inclusions désirées en ajoutant un alliage mère contenant les inclusions le plus tard possible.

5. Alliage de fonte selon la revendication 1, **caractérisé en ce que** l'on forme les inclusions désirées en ajoutant l'alliage mère dans le moule.

6. Alliage de fonte selon la revendication 1, **caractérisé en ce que** l'on forme les inclusions désirées en augmentant la teneur en soufre jusqu'à au moins 0,04 % avant la coulée.

7. Produit en fonte comprenant un alliage selon la revendication 1.

8. Utilisation d'un alliage de fonte selon la revendication 1 pour la production d'un bloc de cylindre.

9. Utilisation d'un alliage de fonte selon la revendication 1 pour la production d'une tête de cylindre.

10. Utilisation d'un alliage de fonte selon la revendication 1 pour la production d'un socle.

11. Utilisation d'un alliage de fonte selon la revendication 1 pour la production d'un logement de transmission ou d'un logement d'essieu.

12. Utilisation d'un alliage de fonte selon la revendication 1 pour la production d'un tambour ou d'un disque de frein.

13. Procédé de production d'une fonte traitée au magnésium, contenant des inclusions qui lubrifient l'insert coupant ou contribuent à la formation d'une couche protectrice sur l'arête coupante, qui comprend les étapes consistant à :
a) préparer un fer de base fondu par des procédés connus en soi,
b) ajouter une quantité fixée à l'avance de magnésium au fer de base fondu et laisser s'établir un équilibre entre le magnésium, l'oxygène et le soufre,
c) ajouter une quantité fixée à l'avance de sulfure de manganèse et/ou de sulfure de molybdène, et finalement
d) couler la masse fondue selon des procédés connus en soi.

14. Procédé de production d'une fonte traitée au magnésium, contenant des inclusions qui lubrifient l'insert coupant ou contribuent à la formation d'une couche protectrice sur l'arête coupante, qui comprend les étapes consistant à :
a) préparer un fer de base fondu par des procédés connus en soi, ledit fer de base contenant au moins 0,1 % de Mn.
b) augmenter la teneur en soufre jusqu'à au moins 0,04 %,
c) ajouter une quantité fixée à l'avance de magnésium, et
d) couler la masse fondue selon des procédés connus en soi.

15. Procédé selon la revendication 13 ou 14, qui comprend en outre la trempe du moule après l'opération de coulée afin de rendre maximale la quantité d'inclusions de sulfure.
